

July 25, 1939.

P. W. LEISNER ET AL

2,167,485

RAIL COOLING

Filed April 20, 1937

3 Sheets-Sheet 1

Fig. 9.



Fig. 1.



Fig. 10.



Fig. 11.



Abscissa represent fillet radii.  
Ordinates represent heat center  
depths magnified 25 times.

INVENTORS

Paul W. Leisner  
Bernard M. Lockard  
By: Cox & Moore ATTORNEYS.

July 25, 1939.

P. W. LEISNER ET AL

2,167,485

RAIL COOLING

Filed April 20, 1937

3 Sheets-Sheet 2

Fig. 2.



Fig. 3.



Fig. 4.



Fig. 5.



Fig. 6.



Fig. 6A.



INVENTORS

Paul W. Leisner  
Bernard M. Lockard  
By: Cox & Moore ATTORNEYS

July 25, 1939.

P. W. LEISNER ET AL

2,167,485

RAIL COOLING

Filed April 20, 1937

3 Sheets-Sheet 3

Fig. 7.



Fig. 8.



INVENTORS

Paul W. Leisner  
Bernard M. Lockard  
Bur-Cout Mfg. ATTORNEYS.

## UNITED STATES PATENT OFFICE

2,167,485

## RAIL COOLING

Paul W. Leisner, Evanston, and Bernard M. Lockard, Oak Park, Ill.

Application April 20, 1937, Serial No. 137,978

7 Claims. (Cl. 238—125)

This invention relates to rails for railroad and like uses, and particularly to a new and improved rail construction, which will cool substantially uniformly without substantial bending or distortion and without undue damage or stress to the metal fibers.

Railroad rails are commonly cooled, as they leave the last set of rolls at the rolling mill in hot plastic condition, by placing them in the air or atmosphere and subjecting them to the cooling action thereof. Due to the symmetry of the rail cross section about its vertical axis, the rail may be depended upon to cool without lateral bending or distortion. However, because of a lack of symmetry of the rail cross section about its horizontal axis, the head and base of the rail do not cool at the same rate. This leads to vertical bending and distortion of the rail during the cooling process. More particularly, with the present and conventional form of rail, the rail base will cool more rapidly than the rail head, leading to the general contraction of the base with respect to the head and the corresponding bending of the rail during the cooling operation.

To compensate for this action rails are commonly deliberately bent from the true and desired alignment by a special set of bending rolls as the rails leave the rolling mill, it being intended that the rail will substantially straighten itself out during the cooling operation. This will be best understood by reference to Fig. 1 of the accompanying drawings wherein the rail is shown in solid lines in the general curved shape which is given to it by this set of special rolls. Initially the entire rail structure is in hot relatively plastic condition. As cooling commences, the base cools more rapidly than the head, and consequently, throughout the cooling, the base is more elastic and stronger than the head. The base will contract with its full elastic force available to combat the efforts of the head which are to enforce less contraction. The head, having less elastic strength, may emerge merely deformed, and this probably explains why most of the cooled rails are straight, as well as shorter (see Fig. 1), instead of merely shorter than the hot rail; but under unfavorable conditions the head may fracture, and this alone seems to account for the so-called "shatter cracks" which recent research has revealed in scattered samples of newly rolled rails.

It may be taken for granted that the uneven cooling of standard shaped rails also accounts for the fact that "gagging" operations are re-

quired to a far greater extent in the manufacture of rails than in the manufacture of symmetrically shaped rolled steel products, and it can hardly be denied that gagging is harmful since it obviously requires stressing the fibers beyond their elastic limits in order to permanently strain the fibers.

Conflicting internal stress and strain of the rail fibers lead to these shatter cracks in the rail structures, which in turn result in "transverse fissures" which frequently develop in conventional rails as they are used in railroad tracks. These transverse fissures were formerly the cause of many railroad disasters and now cause much expense for the detection and replacement of fissured rails.

It is a primary object of the present invention to produce a rail which will have improved cooling characteristics.

It is a further object of the invention to produce a rail structure which will cool uniformly without bending or distortion and without damage or stress to the metal fibers during the cooling operation.

It is a further object of the invention to produce a rail which will cool without bending or distortion, as aforesaid, but which does not sacrifice any of the essential characteristics of the rail.

A further object is to produce a rail which, during and after cooling, will retain the shape which it is initially given as it leaves the shaping rolls, whereby to preserve the rail fibers and to limit gagging operations.

Another object of the invention is to produce a rail having the same depth of heat center in head and base, though the head and base may be of different shape, and to demonstrate how the depth of heat center in the head and base may be relatively proportioned to produce any desired cooling characteristic.

Still another object of the invention is to eliminate the difficulties heretofore discussed in connection with conventional rail cooling.

Other objects and advantages of the invention will be apparent from the following specification, when taken in connection with the accompanying drawings, wherein certain principles and preferred embodiments of the invention are illustrated.

In the drawings, wherein like reference numerals refer to like parts throughout:

Fig. 1 is a diagrammatic view, heretofore referred to, illustrating rail cooling according to conventional methods.

5

10

15

20

25

20

25

30

35

30

35

40

45

50

55

Fig. 2 is an end view of a rail of conventional form.

Fig. 3 is an end view illustrating a rail to which certain features of the invention have been applied.

Fig. 4 is an end view of a rail further improved in accordance with the principles of the invention.

Fig. 5 is an end view of a preferred embodiment.

Figs. 6 and 6A are partial end views of further preferred embodiments of rail heads.

Fig. 7 is a diagrammatic view illustrating the analysis of the invention applied to a rail head.

Fig. 8 is a similar view illustrating the analysis applied to the rail base.

Fig. 9 is a graphical illustration illustrating a comparison of heat center depths.

Fig. 10 is a detail view illustrating the manner in which the rail of Fig. 3 is changed to that illustrated in Fig. 4, and

Fig. 11 is a similar view illustrating the manner in which the rail of Fig. 4 is changed to that illustrated in Fig. 5.

Referring to Fig. 2 of the drawings, there is illustrated a standard 131 pound A. R. E. A. (American Railroad Engineering Association) rail which has been selected for the purpose of analysis. However, it is to be understood that the principles of the present invention are applicable to rails of various shapes and constructions, and is not to be limited to the specific embodiments illustrated.

Reference is now made to the diagrammatic views, Figs. 7 and 8, wherein the head and base respectively of the A. R. E. A. rail are illustrated. One of the manifestations or laws of heat confined within a body placed within a cooling atmosphere, is that the exterior heat radiates to the atmosphere from the body surface, and the interior heat is conducted from the interior of the body to the surface to be radiated in its turn. Another manifestation of heat is that in its conduction through the body it follows the path of least resistance, which, in a homogeneous metal body, is a straight line. In Figs. 7 and 8 the heat center for the head and the bulky portion of the base are indicated by the letter C. These heat centers are the points furthest removed from the exterior surfaces of the rail, in point of heat escape, and their depths determine the ultimate cooling rates of the rail head and base. It will be seen that heat will escape from each heat center through three paths of least resistance. Representing a quantity of heat in any given transverse plane at the heat center, by the length of line T, this heat quantity in the case of the base will escape through two trapezoidal areas 10 and 11 and a rectangular area 12, and in the case of the head through three trapezoidal areas 13, 14 and 15. The area 15 is slightly trapezoidal rather than rectangular due to the curvature of the top of the head. While a rail has length as well as height and width, the conditions of heat escape volumetrically within the rail will be proportional to the conditions of heat escape within any given transverse plane. Hence, for purposes of analysis it is necessary merely to consider the conditions within the given transverse plane, as in Figs. 7 and 8. Also, while the aforementioned trapezoidal and rectangular areas may not define all the possible channels of escape of heat from the heat center, they do represent the relative

resistance against the facilities for escape of heat in the three principal directions and thus do accurately define the relative conditions of heat escape from the heat center. The length T is intended to be a derivative length, but has been magnified in the drawings for purposes of illustration.

The heat center will be that point from which heat may escape in the three principal directions of escape at the same rate. Inasmuch as the derivative quantity of heat represented by the length of the line T escapes through the aforesaid rectangular and trapezoidal areas, and inasmuch as the escape from these areas is limited by their exposed or radiating surfaces, it follows that in the case of the rail base the location of the heat center C will be found by formulating the condition for the rectangular area 12 of heat radiating from its exposed surface 16 in the same space of time in which the trapezoidal area 10 of heat radiates from its exposed surface 17. Expressing this in mathematical relation, T divided by the rectangular area 12 is equal to S divided by the trapezoidal area 10. A solution of this mathematical equation results in the following radiation equation, reference being made to Fig. 8 of the drawings:

Radiation equation:

$$\frac{S}{\text{Trapezoidal area}} = \frac{T}{\text{Rectangular area}}$$

In which:

$$S = T \times R \div \sqrt{A^2 + (B - D)^2}$$

Rectangular area =  $D \times T$ ; and

Trapezoidal area =

$$\frac{\frac{1}{2} \times T \times \sqrt{A^2 + (B - D)^2} - \frac{1}{2} \times S \times R}{2 \times \sqrt{A^2 + (B - D)^2}} = \frac{T \times [A^2 + (B - D)^2 - R^2]}{2 \times \sqrt{A^2 + (B - D)^2}}$$

Hence:

$$\frac{T \times R}{\sqrt{A^2 + (B - D)^2}} = \frac{T}{\frac{T \times [A^2 + (B - D)^2 - R^2]}{2 \times \sqrt{A^2 + (B - D)^2}} \div D \times T} = \frac{T}{D \times T}$$

Or:

$$D^2 - 2 \times (B + R) \times D + A^2 + B^2 - R^2 = 0$$

Or:

$$D = B + R - \sqrt{2 \times R \times (B + R) - A^2}$$

In the foregoing equation R, which is the radius of curvature of the fillet connecting the rail web and rail base, is the only variable, inasmuch as the values for A and B for any given rail design (for example, the 131 pound A. R. E. A. rail) are dependent only upon the value of R and may be determined when R is known. Accordingly the depth of heat center D, which is the measure of the rate of escape of heat from the heat center, is determined by the value of R.

For the head, referring to Fig. 7, substantially the same radiation equation may be made, except that the equation will be changed slightly due to the slight convexity of the top surface 18 of the head. The rail under consideration has a twenty-four inch tread radius which renders the area 15 of slightly trapezoidal shape. In the case of the head the radiation equation is as follows:

Radiation equation:

$$\frac{S}{\text{Lower trapezoidal area}} = \frac{S_1}{\text{Upper trapezoidal area}}$$

In which:

$$S = T \times R \div \sqrt{A^2 + (B - D)^2}; S_1 = T \times 24 \div (24 - D)$$

Lower trapezoidal area

$$\frac{T \times [A^2 + (B - D)^2 - R^2]}{2 \times \sqrt{A^2 + (B - D)^2}}$$

(as for rail base), and

Upper trapezoidal area

$$10 \frac{1}{2} \times 24 \times [24 \times T \div (24 - D)] - \frac{1}{2} \times (24 - D) \times T = \\ T \times [48 \times D - D^2] \div [2 \times (24 - D)]$$

Hence:

$$13 \frac{T \times R}{\sqrt{A^2 + (B - D)^2}} = \frac{T \times 24}{24 - D} \\ \frac{T \times [A^2 + (B - D)^2 - R^2]}{2 \times \sqrt{A^2 + (B - D)^2}} = \frac{T \times [48 \times D - D^2]}{2 \times (24 - D)}$$

Or:

$$20 D^2 - 2 \times \frac{24(B + R)}{24 + R} \times D + \frac{24 \times (A^2 + B^2 - R^2)}{24 + R} = 0$$

Or:

$D =$

$$25 \left[ B + R - \sqrt{2 \times R \times (B + R) - A^2 - \frac{R}{24} \times (A^2 + B^2 - R^2)} \right] \\ + \left( 1 + \frac{R}{24} \right)$$

30 Again it will be seen that the depth of heat center  $D$  for the head, for any given rail design, is dependent solely upon the value of  $R$ , the radius of curvature of the fillet between the head and the web, inasmuch as the values of  $A$  and  $B$  for such given rail design are dependent solely upon the value of  $R$  and are determined thereby.

35 A rail will cool without substantial bending if the head and the base cool at the same rate. The rate at which the web cools is negligible. Inasmuch as the rate at which the rail head and base will cool is determined primarily by the depths of heat centers of these parts, it follows that the rail will cool substantially uniformly and without substantial bending or distortion if the depths of heat centers are the same in the head and base. 40 In the standard 131 pound A. R. E. A. rail, selected for purposes of analysis, and shown in Fig. 2 of the drawings, the radius 26 between the web and base of the rail is three-quarters of an inch. The radius 21 between the rail web and head is one-half inch.

45 By determining the depth of heat center  $D$  for the rail base, for different values of the fillet radius  $R$ , in accordance with the aforementioned equation, it will be found that the depth of heat center materially increases as the fillet radius between the web and base of the rail is decreased. This will best be understood by the graphical illustrations in Fig. 9. For the standard 131 50 pound A. R. E. A. rail, the depth of heat center for the base, using the standard three-quarter inch fillet is 0.957 inch, whereas for a radius of three-eighths of an inch the depth of heat center is increased to 1.017 inches. The heat depth would be further increased by a further reduction of fillet radius, but a radius of three-eighths of an inch is probably the smallest practical and usable radius and hence will be here assumed for the purpose of this analysis as a limiting factor to heat center depth increase by fillet change. By solving the depths of heat center for the rail head, for different values of the fillet radius  $R$ , it will be seen, also referring to Fig. 9, that whereas the depth of heat center for the standard 131 55 pound A. R. E. A. rail with its present one-half

inch fillet radius is 1.218 inches, this heat center depth may be decreased to 1.197 inches by increasing the fillet radius to three-quarters of an inch. As will be seen from the graphical illustration, further increase in the fillet radius of the head results in no further decrease in heat center depth, and increase of the fillet radius beyond seven-eighths of an inch actually results in an increase of heat center depth. The improved rail having a three-eighths inch fillet radius 22 at 60 the base and a three-quarter inch fillet radius 23 at the head is illustrated in Fig. 3.

65 In the improved rail of Fig. 3 the cooling of the base has been materially retarded and the cooling of the head materially increased. However, a further equalization of cooling rates is desirable to produce a rail which will cool uniformly and without bending or distortion. A further reduction of the depth of heat center of the rail head may be effected by changing its shape in 70 the manner illustrated in Fig. 10. This change in design modifies the  $A$  and  $B$  values of the head to facilitate cooling, but does not sacrifice any of the desirable physical characteristics of the standard rail head design. In Fig. 10 the rail head 75 illustrated in Fig. 3 is shown in the dotted outline 25. The solid outline 26 illustrates a modified shape of head wherein an area of metal 27 is removed from the underneath part of the head and arranged at the side of the head in an equal area 80 28. The thus improved rail head is illustrated in Fig. 4. The head fillet radius 23 has been preserved at three-quarters of an inch. However, this rail head, while retaining the most desirable fillet radius, due to its different shaping, will have different  $A$  and  $B$  values, though the value of the fillet radius  $R$  remains unchanged. It will be found, by solving the radiation equation, that the improved rail head of Fig. 4 has a depth of heat center of 1.111 inches, a further substantial reduction and equalization toward the 1.017 inch depth of heat center of the base. This relation is illustrated in the graphical view, Fig. 9. The improved rail head of Fig. 4 has flat surfaces 85 30 (.729 inch wide) on the underneath portions of the head substantially as great as those found in conventional rails, and provide adequate surfaces for the proper seating of splice bars. Also, in this rail the fillet surfaces 31 at the upper portion of the head conform to the shaping of the wheel flange, as will be seen by reference to Fig. 10. This engagement reduces wear of the rail and wheel surfaces as discussed in our Patent No. 2,056,729.

90 The depth of heat center of the head may be still further decreased by changing its shape to that illustrated in Fig. 5. The nature of this change will be best understood by reference to Fig. 11 of the drawings wherein the rail head of Fig. 4 is shown in the dotted outline 35 and the further improved rail head of Fig. 5 is indicated by the solid outline 36. The rail head 36 differs from the head 35 in that its width has been increased one-half inch, the same area of metal in the head being preserved. This widened head, Fig. 5, retains the surfaces of curvature 31 which correspond with the shaping of the wheel flanges, but provides even wider flat surfaces 38 (.881 inch wide) for the seating of splice bars. The curvature of the fillet 23 between the head and the rail web remains the most favorable three-quarter inch radius, but due to the changes in the  $A$  and  $B$  values in this shape of head, the depth of heat center will be found to be 1.031 inches, Fig. 9, substantially the same as the 1.017 inch depth of 95 75

heat center of the base, for all practical cooling purposes. This rail may be depended upon to cool substantially uniformly without substantial bending or distortion or without undue stress to the metal fibers during the cooling process, the rate of cooling in the rail head and rail base being substantially the same. The wide rail head is fully as rugged and strong as conventional rail heads, and provides a greater seating surface for the wheels. The essential characteristics of the rail design are all preserved.

In Fig. 6 there is illustrated a rail head substantially the same as that illustrated in Fig. 5, except that the tread or top surface 40 of the head is flat rather than convex as in Fig. 5, no other changes being made. Such a rail head is well adapted for use with wheels having a cylindrical tread rather than the conventional conical tread. The depth of heat center of this rail head will be found to be 0.991 inch, Fig. 9, or actually less than the depth of heat center of the base, assuming the base fillet to be three-eighths of an inch as in the previously described embodiments. The cooling rates of the head and base are, however, substantially equal for all practical purposes and the rail will cool uniformly and without distortion or stress to the metal fibers. In order to make the cooling rate of the base the same as that of the head, if desired, it will be seen, by reference to Fig. 9, that it is merely necessary to increase the base fillet slightly to substantially seven-sixteenths of an inch.

In Fig. 6A there is illustrated a rail head, which is the same as that illustrated in Fig. 6 except that the fillet radius 24 is so proportioned that the depth of heat center will be 1.017 inches, or the same as that of a rail base with a fillet or three-eighths of an inch. By reference to the cooling curve for the head, Fig. 9, it will be found that fillet 24 will be substantially one-half of an inch.

In accordance with the principles of the present invention, the rail may be so proportioned and shaped as to control or equalize the cooling rates of the head and base. By retarding the cooling of the base and accelerating the cooling of the head, so that the cooling rates are substantially equal, uniform cooling will be effected so that the rail will not be bent or distorted during the cooling process and the metal fibers will not be strained or injured. Gagging is limited. The improved rail, moreover, does not sacrifice any of the essential physical characteristics of the rail and in fact improves them. It retains the desirable characteristics of the head and base shaping.

While the foregoing analysis has referred specifically to a 131 pound A. R. E. A. rail, it is to be understood that the principles of the invention are applicable to rails in general having a wide variation in size and design. It is also to be distinctly understood that the foregoing theory and analysis has been set forth for the purpose of facilitating a better understanding of the principles of the invention, and that the invention, in its broader aspects, is in no sense to be limited thereto or to the accuracy thereof.

Various changes may be made in the invention without departing from the principles thereof. The invention is accordingly not to be limited to the precise embodiments shown and discussed, but only as indicated in the following claims.

The invention is hereby claimed as follows:

1. A rail for railroad and like uses, said rail having a head, a base and a connecting web, said

head being wider and thinner than a standard rail of like weight, the radius of the fillet connecting the rail web and head being increased above that of said standard rail, and the radius of the fillet connecting the rail web and base being decreased below that of said standard rail, whereby to provide a rail having equalized cooling rates in the head and base thereof, and said rail being otherwise of substantially the same general shape as that of said standard rail.

2. A rail for railroad and like uses, said rail having a head, a base and a connecting web, said head being wider and thinner than a standard rail of like weight, and the radius of the fillet connecting the rail web and base being decreased below that of said standard rail, whereby to provide a rail having equalized cooling rates in the head and base thereof, and said rail being otherwise of substantially the same general shape as that of said standard rail.

3. A rail for railroad and like uses, said rail having a head, a base and a connecting web, said head being reshaped as compared with the head of a standard rail of like weight to facilitate cooling, the radius of the fillet connecting the rail web and head being increased above that of said standard rail, and the radius of the fillet connecting the rail web and base being decreased below that of said standard rail, whereby to provide a rail having equalized cooling rates in the head and base thereof, and said rail being otherwise of substantially the same general shape as that of said standard rail.

4. A rail for railroad and like uses, said rail having a head, a base and a connecting web, said head being reshaped as compared with the head of a standard rail of like weight to facilitate cooling, and the radius of the fillet connecting the rail web and base being decreased below that of said standard rail, whereby to provide a rail having equalized cooling rates in the head and base thereof, and said rail being otherwise of substantially the same general shape as that of said standard rail.

5. A rail for railroad and like uses, said rail having a head, a base and a connecting web, said head being wider and thinner than a standard rail of like weight, the radius of the fillet connecting the rail web and head being increased above that of said standard rail to a size imparting a maximum cooling rate to the head, and the radius of the fillet connecting the rail web and base being decreased below that of said standard rail to a minimum practicable size, whereby to provide a rail having equalized cooling rates in the head and base thereof, and said rail being otherwise of substantially the same general shape as that of said standard rail.

6. A rail for railroad and like uses, said rail having a head, a base and a connecting web, said head being provided with a flat tread and being wider and thinner than a standard rail of like weight, the radius of the fillet connecting the rail web and head being increased above that of said standard rail, and the radius of the fillet connecting the rail web and base being decreased below that of said standard rail, whereby to provide a rail having equalized cooling rates in the head and base thereof, and said rail being otherwise of substantially the same general shape as that of said standard rail.

7. A rail for railroad and like uses, said rail having a head, a base and a connecting web, said head being wider and thinner than a standard

5 rail of like weight, the fillet between the tread and the side of the head being shaped to conform to the flange fillet of the wheel with which the rail is designed to cooperate, the radius of the fillet connecting the rail web and head being increased above that of said standard rail, and the radius of the fillet connecting the rail web and base

being decreased below that of said standard rail, whereby to provide a rail having equalized cooling rates in the head and base thereof, and said rail being otherwise of substantially the same general shape as that of said standard rail. 5

PAUL W. LEISNER.  
BERNARD M. LOCKARD.